

April 9, 1929.

A. B. PAGE

1,708,773

PHOTO ELECTRIC CELL

Filed April 27, 1925



Inventor:  
Albert B. Page,

by Alexander S. Lunt.  
His Attorney.

## UNITED STATES PATENT OFFICE.

ALBERT B. PAGE, OF SCHENECTADY, NEW YORK, ASSIGNOR TO GENERAL ELECTRIC COMPANY, A CORPORATION OF NEW YORK.

## PHOTO-ELECTRIC CELL.

Application filed April 27, 1925. Serial No. 25,965.

This application relates to improvements in electrical apparatus, and more particularly to an improvement in photo-electric cells.

5 It is an object of my invention to provide a photo-electric cell which will have a greater efficiency than the type of photo-electric cell which has generally been employed up to the present time.

10 In carrying my invention into effect I roughen the interior surface of the ordinary photo-electric cell by fusing to the glass bulb portion of the cell, numerous small glass particles having the same coefficient of expansion as the bulb. The roughened surface is then given the usual coatings of silver and light sensitive material. I have found that a photo-electric cell thus constructed will give a greater current than a similar cell 15 having a smooth light sensitive surface. While I have not determined the exact cause of the increased current I believe that it is probably due to the fact that a roughened light sensitive surface of given dimensions 20 absorbs more light than a light sensitive smooth surface having similar dimensions.

The novel features which I believe to be characteristic of my invention are set forth with particularity in the appended claims. 25 The invention itself, however, will best be understood by reference to the following description taken in connection with the following drawing in which Fig. 1 is an elevation of a photo-electric cell constructed in accordance with my invention; Fig. 2 is a view partly broken away and on an enlarged scale of a portion of a bulb of a photo-electric cell.

30 Referring to the drawing, I have indicated at 1 a photo-electric cell or container having a bulb portion 2, a neck portion 3, an anode 4, and the usual cathode connection 5. In

the process of manufacture, small glass particles 6 capable of passing through a 40 mesh sieve but retained by a 60 mesh sieve are introduced into the bulb through the neck portion 3. The bulb is then heated and revolved slowly. In this manner the glass particles are evenly distributed over substantially the entire inner surface of the bulb, and fused thereto and to each other. In producing the 45 roughened surface of the cell care should be taken, however, to keep the glass particles away from the smooth window portion 7 of the cell.

50 After the interior surface of the bulb has been roughened, in the manner indicated, the container is evacuated and a coating of silver applied to the roughened surface. A coating of potassium is then applied to the silvered surface and formed by passing a glow discharge in hydrogen. The hydrogen is 55 finally displaced and replaced by argon.

60 What I claim as new and desire to secure by Letters Patent from the United States, is:—

65 1. A photo-electric cell having a roughened surface, a coating of light sensitive material on said roughened surface said coating comprising a cathode, and an anode positioned in photo-electron-receiving relation with respect to said cathode.

70 2. A light sensitive cell including a container, an anode located therein, a plurality of glass particles fused to and projecting from the surface of said container to thereby 75 provide a roughened interior portion, and a coating of light-sensitive material on said roughened portion.

75 In witness whereof, I have hereunto set my hand this 25th day of April, 1925.

ALBERT B. PAGE.